

## UNITED STATES PATENT OFFICE.

VICTOR YNGVE, OF LONG BRANCH, NEW JERSEY, ASSIGNOR TO MANHATTAN ELECTRICAL SUPPLY COMPANY, INC., OF NEW YORK, N. Y., A CORPORATION OF MASSACHUSETTS.

## ELECTRODE.

No Drawing.

Application filed July 30, 1923. Serial No. 654,783.

*To all whom it may concern:*

Be it known that I, VICTOR YNGVE, a citizen of the United States, residing at Long Branch, New Jersey, in the county of 5 Monmouth and State of New Jersey, United States of America, having invented certain new and useful Improvements in Electrodes, do hereby declare that the following is a full, clear, and exact description of the same.

10 This invention relates to new and useful improvements in electrodes for batteries and more particularly to metallic electrodes for dry cells.

15 It is the object of the present invention to provide a metallic electrode which will not be corroded locally before being placed in actual service, the shelf life of which is long, and which is nevertheless inexpensive to manufacture and assemble.

20 It is well known in this art that local corrosion of the metallic electrode is one of the chief reasons for short shelf life. This corrosion is caused by an uneven electrolytic potential on the surface of the electrode, the zinc dissolving in one area being deposited in another, thus pitting the surface, with the result that when the cell is placed in service it is perforated at the thin areas, with resultant loss of electrolyte and ruin of the cell. The uneven electrolytic potential is caused by impurities in the electrode or physical unevenness or strain in the electrode. In zinc cups for dry cells, for instance, it has been found that the zinc is

25 more quickly consumed along seams and at points subjected to excessive strain during the rolling, drawing or other similar operations. Most of this local corrosion is due to local action before the battery is actually

30 placed in service with a consequent lowering of shelf life. In order to improve the efficiency of such batteries it was necessary to use zinc which was relatively free from impurities and great care had to be exercised in drawing or rolling the zinc into sheets and then forming it into cans.

In order to overcome these difficulties, it has been suggested to form cups by casting

or depositing by electrolysis or precipitation. These suggestions were found impractical because too expensive or ineffective materially to improve the efficiency and particularly the shelf life of dry cells. Similarly, dry cells which remain inactive while in stock, the so-called reserve cells, are too expensive or are in other ways objectionable in comparison with the usual type of dry cell.

35 In accordance with the present invention, these disadvantages are avoided by forming the metallic electrodes, e. g. zinc cans of dry cells in the usual manner and then electrolytically depositing thereon a thin film of the same metal, e. g. zinc. This film of metal will be of great purity and will possess a uniform electrical potential and will be free from physical strain. It will therefore resist for a relatively long time the local action to which such electrodes are subjected during the shelf life of a dry cell. The application of such a thin film of electrolytically deposited metal is inexpensive and may entirely replace the now generally practiced amalgamation of the inside surface of zinc cans although, obviously, the present invention may be practiced in combination with the usual amalgamating. While it is desirable that the film of electrolytically deposited metal be as heavy as is permissible from a cost standpoint, any film which covers 40 the surface will give improved results.

45 What I claim is:

1. The method of protecting zinc container electrodes for dry cells against local corrosion, which consists in entirely covering 45 the inside surface thereof with a thin film of zinc electrolytically deposited thereon.

2. The method of making dry cells which consists in first forming the zinc container electrode, then electrolytically depositing on 50 the inside surface thereof a thin film of zinc, and finally completing the dry cell.

55 In witness whereof, I hereunto subscribe my name this 23d day of July 1923.

VICTOR YNGVE.